# EUROPEAN PATENT SPECIFICATION

(11) **EP 0 174 765 B1**
(45) Date of publication and mention of the grant of the patent: **02.11.1989**
(21) Application number: 85306047.3
(22) Date of filing: 27.08.1985
(51) Int. Cl.: B22D 11/06

(54) **Method and apparatus for continuous casting of crystalline strip**
Verfahren und Einrichtung zum Stranggiessen von kristallinen Bändern
Procédé et appareil de coulée continue de bande cristalline

(30) Priority: 13.09.1984 US 650373
(43) Date of publication of application: 19.03.1986
(73) Proprietor: ALLEGHENY LUDLUM CORPORATION, Pittsburgh Pennsylvania 15222 (US)
(72) Inventor: Johns, Robert Harvey, Natrona Heights Pennsylvania 15065 (US); Nauman, John Dana, Natrona Heights Pennsylvania 15065 (US)
(74) Representative: Sheader, Brian N.

(56) References cited:
- US-A- 3 381 739
- US-A- 3 522 836
- US-A- 4 221 257
- US-A- 4 274 473
- US-A- 4 290 476
- US-A- 4 448 236
- US-A- 4 449 568

## Description

This invention relates to a method and apparatus for direct casting or metal alloys from molten metal to continuous strip. More particularly, it relates to feeding molten metal through an open casting vessel outlet to solidify as continuous strip of desired thickness on a moving casting surface.

In conventional production of metal strip, such methods may include the steps of casting the molten metal into an ingot or billet or slab form, then typically includes one or more stages of hot rolling and cold rolling, as well as pickling and annealing at any of various stages of the process in order to produce the desired strip thickness and quality. The cost of producing continuous strip, particularly in as-cast gauges ranging from 0.010 inch to 0.100 inch (0.0254 to 0.254 cm) could be reduced by eliminating some of the processing steps of conventional methods. The as-cast strip could be processed conventionally, by cold rolling, pickling and annealing to final gauges of 0.002-0.040 inch (0.0508 to 1.016 mm).

There are known a wide variety of methods and apparatus for the production of directly cast strip. Typical of such methods are those which include spraying molten metal through a metering orifice across a gap to a rapidly moving quenching surface such as a wheel or continuous belt; methods which partially submerge a rotating quenching surface into a pool of molten metal; methods which use horizontal link belts as quenching substrates upon which molten metal flows for solidification; and methods of casting with twin casting rolls having a pool of molten metal therebetween.

Direct casting of metals through an orifice has long been attempted for the commercial production of strip with good quality and structure. U.S. Patent 112,054 dated February 21, 1871 discloses a method of manufacturing flat solder wire from molten metal forced through an orifice and onto a rotating casting surface. Similarly, U.S. Patent 905,758, issued December 1, 1908, discloses a method of drawing molten metal out of an outlet at the lower end of a vessel and onto a casting surface. British Patent 24,320, dated October 24,1910, discloses a method of producing sheet or strip from molten metal flowing through a tube channel having at least one side in contact with the moving casting surface. Representative of a more recent system in U.S. Patent 3,522,836-King, issued August 04, 1970, which discloses a method of maintaining a convex meniscus projecting from a nozzle and moving a surface past the nozzle orifice outlet to continuously draw off material and solidify as a continuous product. The molten material is maintained in static equilibrium at the outlet and gravitationally maintained in continuous contact with the moving surface. U.S. Patent 4,221,257-Narasimhan, issued September 09, 1980, relates to a method of forcing molten metal under pressure through a slotted nozzle onto the surface of a moving chill body.

US-A-4448 236 upon which the opening portion of claim 1 is based discloses apparatus for producing thin metal sheet wherein molten metal is applied to the peripheral surface of a rotating drum through a nozzle located beneath the drum so that the surface of the drum is moving generally upwardly past the nozzle and which has means for removing the cast metal sheet from the surface of the drum.

The orifice-type casting systems are generally restricted to light gauge materials having a thickness, as-cast, usually of the order of less than about 0.010 inch (0.0254 cm). Such systems appear to be gauge-limited, for the moving quenching surface appears to be limited in the material which it can solidify and carry away as it is delivered from the nozzle orifice. Such systems behave as a molten metal pump and transfer excess molten metal from the orifice to the quenching surface in a molten state with more heat than can be extracted to provide a suitable strip. By reducing the delivery rate of the metal and/or by increasing the velocity of the quenching surface, such a condition can be overcome, however a reduction in gauge will result.

When crystalline strip is attempted to be produced at the high speeds associated with the orifice-type casting systems, poorer quality usually results. As molten metal is sprayed upon a high-speed quenching surface or is flowed out full width on a slower-moving horizontal belt, it rapidly moves away from the source of the supply in a still partially molten state. It is this condition that leads to the deterioration in quality, for as the strip rapidly solidifies from the quenching surface side of the strip, shrinkage occurs which can only be moderated by a fresh supply of molten metal. Without such a fresh supply of molten metal, cracks quickly develop within the structure of the strip and greatly reduce its physical properties. Attempts have been made to improve the nozzle geometry to overcome the problems associated with orifice-type casting as shown in U.S. Patents 4,274,473, issued June 23, 1981 and. 4,290,476, issued September 22, 1981. A disadvantage of the orifice-type casting is that the orifice meters out an amount of molten metal which, in effect, determines the gauge of the strip. Furthermore, relatively high pressure heads used in order to supply enough molten metal to the orifice and a relatively small standoff distance from the casting wheel for containment of the molten metal also limits the strip gauge.

Thicker strip can be produced on a single quenching surface such as by dipping a slowly rotating quenching wheel into a static supply of molten metal to permit the solidification of a much thicker strip. Molten metal solidifies on the surface of this wheel and continues to thicken at a predictable rate until it emerges from this bath of molten metal or it separates from the surface. The fresh supply of molten metal avoids the cracking generally associated with solidification of a finite layer such as in orifice-type casting. Further more, an extremely steep thermal gradient between this molten pool and the solidification front also leads directly to a more uniform internal structure and superior upper surface quality. A drawback from such a dip system comes from the difficulty of keeping molten metal from solidifying upon the edges of the slightly submerged quenching wheel and having a tendency to cast a channel-like structure. Furthermore, there is the added difficulty of ensuring uniform contact between the solidifying strip and the surface of the quenching wheel as it enters the molten pool, and results in poor surface quality on the cast side of the strip. Such difficulties lead to spot variations in strip gauge, wherein lighter gauge sections are produced where intimate contact is reduced or lost.

Other direct casting processes have been proposed, but have not developed into commercial processes. For example, pouring of molten metal on the top of a moving casting wheel produces strip of nonuniform gauge, poor edges and unacceptable quality. U.S. Patent 993,904, dated May 30, 1911, discloses an apparatus including a molten metal first vessel with a gravity discharge outlet opening into the lower part of a tray-like second vessel below the level of molten metal therein. The molten metal passes out of the second vessel through an overflow to deliver molten metal to a casting wheel. U.S. Patent 3,381,739, issued May 7, 1968, discloses a method of forming sheet or strip material by flowing liquid about a surface which is wetted and bridging the distance to the moving casting surface on which it solidifies.

What is needed is a method useful in commercial production for direct casting strip having surface quality comparable to or better than conventionally-produced strip. The method and apparatus of direct casting should produce strip which is superior to orifice-type casting, as well as other known direct casting processes including dip-cast systems, horizontal link belt quenching systems, and twin casting rolls. It is an objective that the method and apparatus overcome the disadvantages of known direct casting methods. Furthermore, what is needed is a method and apparatus to permit the direct casting of relatively thick strip of the order of greater than 0.010 inch (0.0254 cm) and up to about 0.100 inch (0.254 cm) or more. It is desirable that the factors contributing to shrinking and cracking of direct cast strip be minimized or eliminated in order to provide improved surface quality and structure of strip. Furthermore, a method and apparatus is desirable which is suitable for commercial production of strip at reduced cost and to facilitate production of new alloys. The direct cast strip should have good surface quality, edges and structure and properties at least as good as conventionally cast strip.

In accordance with the present invention, a method is provided for directly casting molten metal to continuous strip of crystalline material. The method includes supplying molten metal to a casting vessel having a receiving end and an exit end, the exit end being adjacent and having edges thereof parallel to a casting surface moving generally upwardly past the exit end. The molten metal is fed from the receiving end to the exit end to provide a pool of molten metal having a substantially uniform flow and free upper surface in the exit end. The molten metal flows from the exit end onto the casting surface such that across the width of the exit end of the casting vessel a substantially uniform flow of molten metal is presented to the casting surface. The surface tension of the flowing metal forms all the surfaces of the strip being cast. The top surface tension of the free surface of molten metal pool forms the top of the cast strip, and the surface tension of the molten metal leaving the sides of the exit end forms the edges of the cast strip. The surface tension of the molten metal leaving the bottom of the exit end maintains a meniscus between an inside surface of the bottom of the exit end and the casting surface to form the bottom of the cast strip. The depth of the molten metal in the exit end and distance between the vessel and casting surface are controlled to maintain the surface tension. The as-cast strip is removed from the casting surface.

An apparatus is also provided for directly casting molten metal to continuous strip of crystalline material comprising a movable casting surface, a casting vessel and a means for supplying molten metal to the casting vessel. The casting vessel has a receiving end, an exit end having a generally U-shaped structure adjacent the casting surface and having edges thereof substantially parallel thereto and an intermediate section to facilitate a substantially uniform flow of molten metal from the receiving end to the exit end. The U-shaped structure of the exit end has a bottom wall and diverging inside sidewall surface opening upwardly and having a width between the inside surfaces substantially as wide as the strip to be cast. The exit end has a fixed width along the bottom wall between the inside surfaces and a uniform cross-sectional area over a length sufficient to provide a substantially uniform flow of molten metal from the exit end. The casting surface is movable generally upwardly past the exit end of the casting vessel at a distance of between 0.005 to 0.060 inch (0.013 to 0.152 cm) therefrom at a speed of 20 to 500 feet per minute (6.1 to 152.4 metres per minute).

The present invention will be more particularly described with reference to the accompanying drawings, in which:-
Figure 1 is a schematic of a strip casting apparatus of the present invention,
Figure 2 is an elevation view in cross section of a casting vessel of the apparatus of the present invention,
Figure 2a is a detailed elevation view of Figure 2,
Figure 2b is another detailed view of Figure 2.
Figure 3 is a top view of the casting vessel of Figure 2,
Figure 3a is an end view of the casting vessel of Figure 3,
Figure 4 is an elevation view in cross section of a preferred embodiment of a casting vessel of the apparatus of the present invention,
Figure 5 is a top view of a preferred embodiment of the casting vessel of Figure 4,
Figure 6 is an enlarged elevation view of a preferred embodiment of the exit end of a casting vessel of the apparatus of the present invention,
Figure 7 is a photomicrograph of typical Type 304 alloy as-cast strip of the present invention, and
Figure 8 is a photomicrograph of a typical Type 304 alloy conventionally produced hot-rolled ban.
Figure 1 generally illustrates casting apparatus 10 including transfer vessel 12 and feed tundish 14 for supplying molten metal to casting vessel 18 for directly casting molten metal on a casting surface 20 to produce continuous product in strip or sheet form 15. Molten metal 19 is supplied from vessel 12 to tundish 14 to casting vessel 18 in a conventional manner. Stopper rod 16 or other suitable means may control the flow of molten metal to casting vessel 18 such as through spout 17.

Casting vessel 18 is shown substantially horizontal having a receiving end and an exit end disposed adjacent to the casting surface 20.

The supply of molten metal 19 through the casting vessel 18 may be accomplished by any suitable conventional methods and apparatus of vessels, tundishes, or molten metal pumps, for example. Vessel 12 and feed tundish 14 may be of known design and should be suitable for supplying an adequate amount of molten metal to casting vessel 18 for strip generation at the casting surface.

Casting surface 20 may also be conventional and may take the form of a continuous belt, or a casting wheel. Preferably a casting wheel is used. The composition of the casting surface does not appear to be critical to the present invention, although some surfaces may provide better results than others. The method and apparatus of the present invention have been used with casting surfaces of copper, carbon steel and stainless steel. It is important that the casting surface be movable past the casting vessel at controlled speeds and be able to provide desired quenching rates to extract sufficient heat for solidifying the molten metal into strip form. The casting surface 20 is movable past casting vessel 18 at speeds which may range from 20 to 500 feet per minute (6.1 to 152.4 metres per minute), preferably 50 to 300 feet per minute (FPM) (15.24 to 91.44 metres per minute), which is suitable for commercial production of crystalline material. The casting surface 20 should be sufficiently cool in order to provide a quenching of the molten metal to extract heat from the molten metal for solidification of strip of crystalline form. The quench rates provided by casting surface 20 of apparatus 10 are less than 10,000°C per second and typically preferably less than 2000°C per second.

Two important aspects of the casting surface and casting vessel are that the casting surface have a direction of movement generally upwardly past the exit end of vessel 18 and the vessel 18 a free surface molten metal pool in exit end 26. The free surface of the molten metal pool in exit end 26 is essential to development of good top surface quality of the cast strip. By "free", it is meant that the top surface is unconfined by structure, i.e., not in contact with vessel structure and free to seek its own level between receiving section 22 and exit end 26. Generally, the path is oriented at an included angle 6 (Figure 2a) from about 0° to 135° from the horizontal and in the direction of metal flow as measured between the direction of metal flow at the free surface of molten metal in the exit end and the direction of movement of the casting surface at the free surface in the exit end of casting vessel 18. For a casting wheel, the path of the casting surface is tangent to the free surface at the exit end of vessel 18. Preferably, the angle is between 0° and 45° from the horizontal. For a casting wheel, preferably, the vessel is adjacent a position in an upper quadrant of the wheel when the free surface of molten metal is near the crown of the casting wheel, the angle is at about the 0° position.

Casting vessel 18 is essential to the method and apparatus 10 of the present invention and is better shown in Figure 2 which is an elevation view of the vessel 18. Casting vessel 18 is disposed adjacent casting surface 20, preferably is substantially horizontal, and is composed of heat insulative and refractory material described below. This arrangement is necessary for providing the required uniform and fully-developed flow of molten metal to the casting surface 20. Vessel 18 includes a receiving end 22 at a rearward section and an exit end 26. Preferably, receiving end 22 and exit end 26 have substantially the same cross-sectional area or exit end 26 has a greater cross-sectional area as measured perpendicular to the direction of metal flow from the receiving end 22 to exit end 26. Receiving end 22 is shown deeper than exit end 26 which facilitates receiving molten metal 19 such as from supply spout 17 and for developing a flow of molten metal to exit end 26.

Exit end 26 of vessel 18 has a generally U-shaped structure defined by a bottom wall portion 28 and sidewalls 30, as is shown in Figure 3. Sidewalls 30 may have vertical inside surfaces 31, but preferably, the surfaces 31 of sidewalls 30 of the U-shape structure diverge to open upwardly to facilitate metal flow. The slight taper tends to improve metal flow from exit end 26, but too great a taper may cause a loss of surface tension control and flooding of molten metal. A taper of less than 10° per side and preferably 1-5° is provided.

Exit end 26 includes bottom wall 28 which has a generally planar inside portion having a length sufficient to provide a substantially uniform flow of molten metal from the exit. Preferably, the length of the planar wall portion as measured in the direction of metal flow is at least equal to the depth of molten metal pool to be contained in exit end 26. More preferably, the ratio of length to depth is at least 1:1 or greater. Exit end 26 preferably has fixed or uniform dimensions of width and height throughout the length of the planar inside surface of bottom wall 28 to define a uniform cross-sectional area in exit end 26. The width of the exit end 26 as measured between the inside surfaces 31 of sidwalls 30 along the free surface of molten metal pool is substantially as wide as the strip to be cast. Preferably, exit end 26 is positioned adjacent casting surface 20 with the ends or edges of the sidewalls 30 and bottom wall 28 defining the U-shaped structure being substantially parallel to the casting surface.

To facilitate transition flow between receiving section 22 and exit end 26, an intermediate section 24 communicating between the receiving end 22 and the exit end 26 should be provided in order to have a substantially uniform flow at exit end 26. Preferably, intermediate section 24 maintains substantially uniform cross-sectional area throughout its length from receiving section 22 to exit end 26. Intermediate section 24 shown in Figure 3 has a gradually increasing width from the receiving end 22 to exit end 26 and, as shown in Figure 2, a gradually decreasing depth so as to maintain a substantially uniform cross-sectional area throughout its length. Intermediate section 24 may be provided with a tapered bottom wall 32 which gradually decreases the depth of the vessel 18 from the receiving end 22 to the exit end 26. Similarly, intermediate section 24 may have at least one sidewall 34 which fans outwardly in order to provide a gradually increasing width from the narrower receiving end 22 to the wider exit end 26. Figure 2 is a top view of casting vessel 18 illustrating the widening of sidewall 34 of intermediate section 24.

Figure 2 also illustrates that weirs or weir plates 36 may be used in casting vessel 18 such as in an intermediate section 24 or near where section 24 merges into exit end 26 in order to further facilitate development of uniform flow. Weir plates 36 should be made of a refractory or heat-resistant material which is also resistant to corrosion by molten metal. Kaowool refractory board, treated with a diluted coloidal silica suspension has proven satisfactory. Weirs 36 may extend across the entire width or a portion of the width of casting vessel 18. As shown in Figure 2, preferably, the molten metal level in the receiving end 22 of casting vessel 18 is at about the same level as the molten metal in exit end 26. Weirs 36 are useful for baffling or dampening the flow in order to facilitate development of a uniform fully-developed flow and to restrain movement of surface oxides and slag.

Figures 2a and 2b illustrate the use of surface tension of the flowing molten metal to form the surfaces of the strip being cast. Figure 2a is a detailed elevation view in partial cross section of exit end 26 adjacent casting surface 20. Molten metal flowing from the exit end 26 forms and maintains a meniscus 35 between the inside surface of bottom wall 28 of the U-shaped structure and the casting surface. The surface tension forming meniscus 35 forms the bottom of the strip 15 being cast. The surface tension of the free surface of the molten metal pool in exit end 26 forms a curvilinear portion 39 on the top of the molten metal in the U-shaped structure as it forms the strip product.

Figure 2b illustrates exit end 26 adjacent casting surface 20 showing solidifying metal 19 therebetween in a view from under exit end 26. The surface tension of the molten metal 19 forms the convex surfaces or meniscus 37 between exit end 26 and casting surface 20 at the inside surface 31 of sidewalls 30 near bottom wall 28.

A preferred embodiment of casting vessel 18 is shown in the elevation and top views of Figures 4 and 5, respectively. Vessel 18 is shown having an outer metal support shell 38, a refractory insulation 40, and a liner 42 which defines the internal surface of the casting vessel 18 and which is in contact with molten metal during casting. The construction of vessel 18 should be made from refractory material which is heat insulative and resistant to molten metal corrosion. The casting vessel may be secured to some suitable table or means to orient and position the vessel at the desired casting position relative to the casting surface or wheel 20. The exit end 26 of casting vessel 18 should have the front face or edges 33 of sidewalls 30 and bottom wall 28 which define and form the U-shaped structure contoured to the casting. surface. This can be done simply by using 60 or 100-grit silicon carbide grinding paper held between the casting surface and the vessel assembly and rubbing the paper against the vessel 18 to make the edges parallel to the wheel. The front surface of the casting vessel 18 may then be brush coated with zirconia cement and allowed to dry before casting.

Figures 4 and 5 illustrate a preferred embodiment of the casting vessel 18 of the present invention which is useful for casting strips of 4 inches (10.16 cm), and up to about 13 inches (33.02 cm) wide and may be useful up to 48 inches (121.92 cm) wide. The metal support shell 38 may be used depending upon the type of material used for the insulation layer 40. Insulation layer 40 may be a foamed ceramic cement insulation which would need an external support such as a metal support shell 38. In the alternative, if a standard refractory brick or block is used and cemented together into the desired shapes and then carved to achieve the desired inner and outer dimensions, then the outer shell 38 is not necessary. The vessel 18 may also be a monolithic shape formed from castable ceramic material. Liner 42 on the internal surface of casting vessel.18 is also made of an insulating refractory molten metal resistant material. It has been found that an insulating blanket of a high alumina fiber-silicate composition is useful, such as Fiberfrax brand material, that has been saturated in a diluted colloidal silica suspension and contoured within the casting vessel 18 and then dried prior to actual use.

Figures 4 and 5 also show a rear overflow element 44 including a rearwardly-sloping surface extending from the inner surface of casting vessel 18 to the outer walls of vessel 18. The height of the overflow element 44 determines the maximum depth of molten metal that may be contained in the receiving end 22 and, accordingly, the depth of the molten metal in the exit end 26 of casting vessel 18. Overflow element 44 facilitates control of the molten metal level in the casting vessel 18 which is essential to gauge and quality control of the cast strip.

Also shown in Figure 4 is a casting vessel 18 which may optionally include a cover assembly 46 in the vicinity of intermediate section 24 of casting vessel 18. Cover 46 includes downwardly-extending walls 48 and 50 joined by a bottom surface 52. The downwardly-extending walls 48 and 50 are similar to the weir plates shown in Figure 2. Cover 46 is generally composed of a refractory insulative material resistant to molten metal. Cover 46 may comprise a liner, a refractory insulation layer and an outer metal shell similar to the liner 42, refractory insulation layer 40 and outer metal shell 38 of casting vessel 18. The cover 46 may extend across the entire width of part of the width of casting vessel 18 in the vicinity of intermediate section 24. It is important that the presence of a cover 46, which is useful for retaining the heat in the molten metal in the casting vessel 18, does not contact the molten metal in the receiving end 22 and exit end 26 in order to maintain the free surface in the pool in exit end 26. The cover also can extend over portions or all of rear receiving section 22 to contain a protective atmosphere therein.

Figure 6 illustrates another embodiment wherein the exit end 26 of vessel 18 is provided with a means for providing a non-oxidizing atmosphere in a zone defined above the molten metal across the width of the U-shaped structure of the exit end adjacent to the casting surface 20 together with a means for radiantly cooling the molten metal in that zone. The two features may be present separately or in combination.

Means for providing a non-oxidizing atmosphere provides a protective cover or blanket of inert or reducing gases in a zone about the molten metal in the U-shaped structure of exit end 26. The gases minimize or prevent the build-up or formation of slag and oxides on the top surface of the molten metal, which oxide could be cast into the cast strip. The non-oxidizing atmosphere may be static, or a recirculating atmosphere. Preferably, a non-contacting cover over the zone above the molten metal pool at the exit end 26 of casting vessel 18 and at least one gas nozzle or a series of nozzles 56 provides a continuous flow of inert or reducing gas counter to the direction of the cast strip. Preferably the gas is introduced so that it impinges in the zone on the top of the molten metal liquid pool where the strip is emerging. The embodiment may provide a protective cover for sealing the zone over the molten metal pool containing a blanket of inert or reducing gases directed into streams of gases to push any oxide away from the forming of the strip. The series of narrow gas nozzles 56 is positioned along the width of the casting strip so that streams or jets of gas impact the zone wherein the strip emerges from the liquid pool. Nozzles 56 are directed counter to the casting of the strip at an angle to the plane of the formed strip, preferably about 20°―30°. The gas blanket may be a gas selected from hydrogen, argon, helium, and/or nitrogen in order to minimize the oxides that may be formed during casting. The velocity of the gases from nozzle 56 should be quite low, for higher velocities may cause a disturbance in the upper surface of the molten metal pool and result in damage to the cast strip.

Means for radiantly cooling the molten metal in the zone may include providing a coolant in the vicinity of the zone to facilitate extraction of heat from the top surface of the molten metal. The coolant may be provided by a panel of tubes or pipes 54 located above the molten liquid to remove radiated heat from the molten metal. Water or other fluid may be used as a coolant. Preferably, a cover is provided which includes a series of water-cooled tubes 54 sealed to the top of the casting vessel 18 with refractory material and cement. Radiant cooling of the top surface of molten metal as it flows from the U-shaped structure of exit end 26 onto the casting surface improves the heat extraction from the top surface of the solidifying molten metal to improve as-cast strip top surface quality and structure by controlling the growth of dendritic structure in the strip.

Preferably, means for providing a non-oxidizing atmosphere and the means for radiantly cooling are used in combination. A non-contacting cover for sealing the zone over the molten metal at the exit end 26 includes a cooling means to remove radiated heat from the molten metal and a non-oxidizing atmosphere means. Preferably, the cover includes a series of water-cooled tubes 54 and a series of gas nozzles 56. The inert gases in this embodiment are cooled by the tubes 54 which further facilitate removal of the radiant heat. The cover containing the cooling tubes 54 seals the zone to reduce oxide or slag formation which could be deposited on the strip product.

In the operation of the casting apparatus of the present invention, vessel 12, tundish 14 and casting vessel 18 are preheated to operating temperatures prior to introducing molten metal into the casting vessel 18 for the production of strip material. Any conventional heating means should be suitable and may be used. An air-acetylene or air-natural gas heating lance positioned in the receiving end 22, as well as providing a preheat front cover for the front edges of the casting vessel U-shaped structure which will be placed adjacent the casting surface 20. Normal preheating temperatures for casting molten stainless steel may be of the order of 1900-2000°F (10381093°C). After the minimum preheat levels desired are reached, the heating lances are removed and the vessel 18 is positioned adjacent the casting surface at a preset standoff distance such as between 5 and 20 mils (0.127 and 0.508 mm).

In commencing the method of directly casting alloy from molten metal to continuous strip, molten metal 19 is supplied from a bulk transfer ladle or vessel 12 to a feed tundish 14 and thereafter to the casting vessel 18 which is oriented substantially horizontally. The flow of molten metal from feed tundish 14 to casting vessel 18 may be controlled and regulated by valve means such as stopper rod 16 and through spout 17 into the rear feed section or receiving end 22 of casting vessel 18. As vessel 18 begins to fill with molten metal, the molten metal begins to flow in a direction toward the exit end of the vessel and flows through an intermediate section 24 and the exit end 26 as shown in Figure 2. Casting vessel 18 permits the molten metal to flow so as to feed the molten metal to the exit end 26 of vessel 18. Casting vessel 18 may include wires 36 such as shown in Figure 2 to dampen and baffle the flow of molten metal 19 in order to facilitate a uniform fully-developed flow in exit end 26. The molten metal preferably maintains a substantially uniform cross-sectional area of flow from the receiving end 22 through the exit end 26. Generally exit end 26 is wider than the receiving end 22 and the U-shaped structure has a width which approximates the width of the strip to be cast. Casting vessel 18 has a casting volume having tapered and fanned intermediate section. Casting vessel 18 is designed to prevent cross flows of molten metal within the vessel while developing a uniform turbulent flow from exit end 26 across the width of the U-shaped structure in end 26 such that the fully-developed flow has the bulk of the velocities in the direction of flow from the receiving end 22 to the exit end 26. The level of molten metal in exit end 26 is about the same as the level in receiving end 22, although the depth of the molten metal will be less in exit end 26. The molten metal continues to flow from the exit end 26 onto the moving casting surface 20 such that across the width of the U-shaped structure of exit end, a substantially uniform flow of molten metal is presented to the casting surface 20. The molten metal in exit end 26 has a top surface tension and the molten metal leaving the opening has edge surface tension which form, in part, the top and edges, respectively, of the cast strip 15. The bottom surface is formed from surface tension in the form of a meniscus between the bottom inside surface of the U-shaped structure and the casting surface.

Though there is no intent to be bound by theory, it appears that the solidification of the molten metal leaving the exit end of vessel 18 commences with the molten metal contacting the casting surface as it leaves the bottom of the U-shaped opening of exit end 26 of vessel 18. The strip is solidified from the pool of molten metal available to the casting surface at the exit end of vessel 18 and forms a thickness wherein the solidifying strip is continually presented with an oversupply of molten metal until leaving the exit end 26 of vessel 18. Such a pool of molten metal is believed to form a substantial part of the strip thickness as it contacts the moving casting surface 20 with only a minor portion of the strip thickness resulting from molten metal solidified as it was pulled out of the vessel 18 adjacent the top curvilinear surface tension portion 39. It is estimated that more than 70% and probably more than about 80% of the strip thickness results from the pool of molten metal provided adjacent the meniscus 35. The molten metal solidifies from the bottom of the molten metal pool provided to the casting surface from the bottom of the U-shaped structure of exit end 26 of vessel 18.

Casting surface 20 moves past casting vessel 18 in a generally upward direction from the bottom of the U-shaped opening of exit end 26 to the open top of the opening. The position of vessel 18 on the casting surface 20 and the speed of the casting surface are predetermined factors in order to achieve the quality and gauge of the cast strip. If the casting surface 20 is a casting wheel, then the vessel 18 is positioned, preferably, on an upper quadrant of the casting wheel.

By the method of the present invention, there is an important control of several factors which results in the ability to cast desired gauges of metal strip ranging from 0.01 to 0.06 inch (0.0254 to 0.1524 cm) with good surface quality, edges and structure. The control of molten metal flow onto the casting surface, the speed of the casting surface, the solidification from the bottom of the molten metal pool, and the controlled depth of molten metal in the pool and standoff distance from the casting surface to maintain the surface tension of the molten metal are important interrelating factors.

In order to better understand the present invention, for following examples are presented.

### Example I

A casting vessel having the structure generally as shown in the Figure 2 but having only one weir plate 36 near the exit end 26 was constructed from hardened blocks of Kaowool refractory, which is an alumina-silica composition material. It was treated by soaking it with a colloidal silica suspension dried overnight at 250°F (121°C) and then fired for 1 hour at 2000°F (1093°C) in air. After the blocks were cut and shaped, they were coated with a thin layer of Kaowool cement. The vessel was shaped to the contour of the wheel and then the U-shaped structure ends were coated with a thin layer of a zirconia cement. A weir of similar composition was used. The casting vessel was then heated with air-acetylene lances. The vessel 18 was about 8.75 inches (22.23 cm) long from the receiving end 22 to the exit end 26 and was about 6.5 inches (16.5 cm) wide at the receiving end 22 and about 4 inches (10.16 cm) wide at bottom wall 28 and exit end 26. Molten metal of Type 304 alloy was tapped at 1580°C, supplied to the vessel 18 and maintained at a level of about 1.75 inches (4.45 cm) deep in the receiving end 22 and the molten metal was about 0.75 inches (1.9 cm) deep in the U-shaped structure in the exit end 26 of vessel 18. A casting surface was a copper casting wheel having a width of 7 inches (17.78 cm) and a diameter of about 36 inches (91.44 cm) which provided cooling of the order of less than 2000°C/sec. The casting wheel was rotated at a speed of about 2050 to 300 feet per minute (76.2 to 91.44 metres per minute) past the exit end of vessel 18 and spaced about 40 mils (1.016 mm) therefrom at an angle 0 of about 40°. The U-shaped structure of the vessel had diverging or tapered inside surface 31 of sidewalls 30 of exit end 26 opening upwardly. The taper was of the order of about 3° per inside surface. Run 25 of about 100 pounds (45.36 kg) was cast according to the present invention and resulted in successful production of strip having a width of about 4 inches (10.16 cm) and a uniform thickness of from 16 to 18 mils (0.406 to 0.457 mm) having smooth and uniform upper and lower surface as-cast and flat edges showing no signs of raggedness or curls.

### Example II

A casting vessel having a structure generally as shown in Figure 4 was constructed having a Kaowol refractory and alumina bubble refractory insulation 40 in a metal shell 38. The liner 42 was made of Fiberfrax material, 0.5 inch (1.27 cm) thick at eight pounds per cubic foot (128.14 kg/m³) which was saturated with a diluted colloidal silica suspension and then dried prior to use. The vessel 18 outside dimensions were about 15 inches (38.1 cm) long and 18 inches (45.72 cm) wide at the exit end and vessel 18 had a slight increasing cross-sectional area to exit end 26. Weir plate 36 was made and positioned similar to Example I and cemented between sidewalls of vessel 18. The inside surfaces 31 of sidewalls 30 were also tapered or diverging of the order of about 3° per surface. The casting vessel was set at a standoff distance of about 35 mils (0.89 mm) at an angle of about 0° for the free surface of the molten metal was near the crown of the casting wheel. A 500-pound (226.8 kg) Run 84-97 of molten metal of Type 304 was cast according to the present invention on a casting surface of a low carbon steel seamless pipe having a 12.75-inch (32.39 cm) outside diameter, a 0.375-inch (0.95 cm) wall thickness, 48 inches (121.92 cm) wide and internally spray water cooled. The casting wheel was rotated at about 200 FPM (60.96 metres per minute) at the start of the casting for 10-15 seconds to facilitate flushing of the initial metal flow and then slowed to 100 FPM (30.48 metres per minute) for the duration of the Run. The molten metal maintained a depth of about 2 inches (5.08 cm) in the exit end 26 and 2.75 inches (6.98 cm) in the receiving end 22.

The vessel 18 also included a cover having a means for radiantly cooling and means for providing a helium atmosphere as shown in Figure 6. The cooling was effected by circulated water at about 3 gallons (13.64 litres) per minute through copper tubing having a 0.375-inch (0.95 cm) outside diameter.

The as-cast strip was about 13 inches (33 cm) wide, and having a uniform thickness of about 45 mils (1.143 mm) and having good upper surface quality which was uniform, smooth and crack free. The as-cast strip was then conventionally processed by-pickling in a nitric/hypofluoric acid, cold rolling about 50% reduction, annealing at 1950°F (1065°C) for 5 minutes, pickling again in a similar manner, and then cold rolling to 5 mils (0.127 mm) and annealed. The room temperature mechanical properties of the annealed as-cast samples are shown below in comparison to typical properties of conventionally produced Type 304 annealed hot-rolled band.

Type 304 alloy conventionally produced may have typical or average room temperature mechanical properties of annealed hot-roll band of 10.1 KSI (7.0 bar) tensile strength, 43.8 KSI (3.0 bar) yield strength and 57% elongation in 2 inches (5.08 cm).

Figure 7 is a photomicrograph of as-cast strip of the present invention showing the typical internal structure from Run 84-52. The Type 304 alloy, shown at 100x magnification, illustrates the typical as-cast structure of small columnar cells oriented in the direction of strip thickness, i.e., top to bottom surfaces. This direction generally conforms to the direction of heat extraction from the strip as it solidifies. The method and apparatus of the present invention controls the growth of the dendritic structure in the strip to produce an as-cast strip which can be conventionally processed into finished strip having properties comparable to or better than conventionally produced strip product.

Figure 8 illustrates a typical structure of a conventionally produced hot-roll band of type 304 alloy at 100x magnification.

It is observed that the method and apparatus of the present invention results in even better strip structure and quality as the gauge of the strip product increases and as the width of the strip increases. The tendency of edge curl in the strip product cast in 4 to 6-inch (10.16 to 15.24 cm) widths appears to no longer be present in the wider widths up to 13 inches (33.02 cm). The method and apparatus of the present invention provides an uncomplicated and direct method for casting crystalline metal strip or sheet from molten metal to continuous strip. The shrinking and cracking problems of finit film solidification are eliminated and a relatively thick strip of quality comparable to or better than conventional production methods is provided.

The method and apparatus appear useful for various metals and alloys, including stainless steel and silicon steels.

## Claims

1. A method of directly casting molten metal to continuous strip or crystalline metal, comprising supplying molten metal (19) to a casting vessel (18), moving a cooling casting surface (20) generally upwardly past an exit of the casting vessel, flowing molten metal from the exit onto the moving casting surface, the surface tension of the free surface of the molten metal maintaining a meniscus (35) between the exit and the casting surface, and removing the cast strip (15) from the moving casting surface, characterised in:
the casting vessel (18) having a receiving end (22) and an exit end (26), the exit end (26) being adjacent to the casting surface (20) and having edges (33) thereof parallel to the casting surface (20);
feeding molten metal from the receiving end (22) to the exit end (26) to provide a pool of molten metal having a substantially uniform flow and a free upper surface in the exit end (26) of the casting vessel (18);
flowing molten metal from the exit end (26) onto the moving casting surface (20) with a substantially uniform flow across the width of the exit end (26), the surface tension of the flowing metal forming all the surfaces of the strip to be cast, the surface tension of the free surface of the molten metal pool forming the top of the cast strip, the meniscus (35) forming the bottom of the cast strip; the surface tension of the molten metal leaving two sides (30) of the exit end (26) forming the edges of the cast strip and being substantially as wide as the strip being cast; and
controlling the depth of molten metal in the exit end (26) of the vessel (18) and the distance between the exit end (26) and the casting surface (20) to maintain the surface tension of the molten metal on the top, bottom and sides.

2. A method according to claim 1, wherein the feeding of molten metal (19) from the receiving end (22) to the exit end (26) includes maintaining a substantially uniform cross-sectional area of flow in the exit end (26).

3. A method according to claim 1 or 2, wherein the feeding of molten metal (19) includes maintaining a substantially uniform cross-sectional area of flow from the receiving end (22) through the exit end (26).

4. A method according to claim 1, or 3, wherein said feeding of molten metal (19) in the casting vessel (18) includes providing molten metal in the receiving end (22) at the same level as in the exit end (26).

5. A method according to any one of the preceding claims wherein said feeding the molten metal (19) includes having a gradually increasing width of flow from the receiving end (22) to the exit end (26) while maintaining a substantially uniform cross-sectional area of flow.

6. A method according to any one of the preceding claims including baffling the flow of molten metal in the casting vessel (18) to facilitate development of uniform flow at the exit end (26).

7. A method according to any one of the preceding claims, including moving the casting surface (20) past a generally U-shaped structure of the exit end (26) of the vessel (18) in a direction generally from the bottom of the U-shaped structure to the top of the exit end (26).

8. A method according to any one of the preceding claims, including moving the casting surface (20) in a path from the horizontal and in the direction of the metal flow at an angle of from 0° to 135° as measured between the free surface and the casting surface direction at the exit end (26) of the vessel (18).

9. A method according to claim 8, wherein the angle is from 0° to 45° from the horizontal.

10. A method according to any one of the preceding claims, including controlling the thickness of the strip (15) by the speed of the casting surface (20) and the depth of molten metal (19) in the exit end (26) of the casting vessel (18).

11. A method according to any one of the preceding claims, including cooling the molten metal after contact with the casting surface (20) at a rate of less than 2000°C per second to effect solidification of crystalline metal.

12. A method according to claim 11, wherein the cooling is at a rate of less than 1500°C per second.

13. A method according to any one of the preceding claims, wherein the casting surface is moved at a speed of 20 to 500 feet (6.096 to 152.4 metres) per minute.

14. A method according to any one of the preceding claims, including providing the casting surface (20) parallel to edges (33) of the exit end (26) and at a distance of between 0.005 to 0.060 inches (0.127 to 1.524 mm) from the exit end (26).

15. A method according to any one of the preceding claims, including removing strip (15) from the casting surface (20) having a uniform strip width, which ranges from 4 to 48 inches (10.16 to 121.92 cm).

16. A method according to any one of the preceding claims, including removing strip (15) from the casting surface (20) having a uniform thickness which ranges from 0.010 to 0.100 inch (0.254 to 2.54 mm).

17. A method of directly casting molten metal to continuous strip of crystalline metal, comprising supplying molten metal (19) to a casting vessel (18), moving a cooling casting surface (20) generally upwardly past an exit of the casting vessel, flowing molten metal from the exit onto the moving casting surface, the surface tension of the free surface of the molten metal maintaining a meniscus (35) between the exit and the casting surface, and removing the cast strip (15) from the moving casting surface, characterised in:
the casting vessel (18) being substantially horizontal and having a receiving end (22) and an exit end (26), the exit end (26) being adjacent to a casting surface (20) and being generally U-shaped with edges (33) thereof parallel to the casting surface (20) and spaced therefrom at a distance of between 0.005 to 0.060 inch (0.127 to 1.524 mm);
moving the casting surface (20) generally upwardly past the exit end (26) at a speed of 20 to 500 feet (6.096 to 152.4 metres) per minute in a path at an angle of 0° to 135° as measured between the free surface in the direction of metal flow and the direction of the casting surface (20) at the exit end (26) of the casting vessel (18);
feeding molten metal (19) from the receiving end (22) to the exit end (26) while maintaining a substantially uniform cross-sectional area or greater of flow to provide a pool of molten metal having a substantially uniform flow and free upper surface in the exit end (26);
flowing molten metal (19) from the U-shaped structure of the exit end (26) onto the moving casting surface (20) with a substantially uniform flow across the width of the exit end (26), the surface tension of the flowing metal forming the surfaces of the strip (15) being cast, the surface tension of the free surface of the flowing molten metal forming the top of the cast strip, the surface tension of the molten metal leaving two sides (30) of the exit end (26) forming the edges of the cast strip and being substantially as wide as the strip (15) being cast and the surface tension of the molten metal leaving the bottom of the U-shaped structure maintaining the meniscus (35) between an inside surface of the bottom (28) of the exit end (26) and the casting surface (20) to form the bottom of the cast strip (15);
cooling the molten metal upon contact with the casting surface (20) at a rate of less than 2000°C per second to effect solidification of crystalline metal; and
controlling the depth of molten metal in the exit end (26) of the vessel (18) and the distance between the exit end (26) and the casting surface (20) to maintain the surface tension of the molten metal on the top, bottom and sides.

18. Apparatus for directly casting molten metal to continuous strip of crystalline material, comprising a casting vessel (18) having an exit (26) and a casting surface (20) movable generally upwardly past the exit (26) characterised in:
the casting vessel (18) having a receiving end (22); a generally U-shaped exit end (26) and an intermediate section (24) therebetween;
means (12) for supplying molten metal (19) to the receiving end (22) for the casting vessel (18);
said casting vessel (18) having its exit end (26) adjacent the casting surface (20) and edges (33) thereof substantially parallel to the casting surface (20), the intermediate section (24) facilitating a substantially uniform flow of molten metal (19) from the receiving end (22) to the exit end (26), the U-shaped exit end (26) having a planar bottom wall (28) and diverging inside sidewalls (31) opening upwardly and having a width between the inside surfaces substantially as wide as the strip (15) to be cast, the exit end (26) having fixed width along the bottom wall (28) between the inside surfaces (31) of the sidewalls (30) and a uniform cross-sectional area over a length sufficient to provide a substantially uniform flow of molten metal from the exit end (26);
said casting surface (20) being movable generally upwardly past the exit end (26) of the casting vessel (18) at a distance of between 0.005 to 0.060 inches (0.127 to 1.524 mm) therefrom and at a speed of20.to 500 feet (6.096 to 152.4 metres) per minute.

19. Apparatus according to claim 18, including a casting vessel (18) wherein the molten metal level in the receiving end (22) and exit end (26) are at the same level.

20. Apparatus according to claim 18 or 19, wherein the intermediate section (24) communicating between the receiving end (22) and exit end (26) has a gradually increasing width at the exit end (26) avd a gradually decreasing depth so as to maintain a substantially uniform cross-sectional area throughout the length of the casting vessel (18).

21. Apparatus according to claim 18,19 or 20, including baffles (36 or 48, 50) in the casting vessel (18) to facilitate development of uniform flow.

22. Apparatus according to any one of the preceding claims 18 to 21, wherein the casting surface (20) has a direction of movement upwardly from the horizontal and direction of metal flow at the free surface of molten metal at the exit end (26) oriented at an angle of from 0 to 135° from the horizontal between the free surface and the casting surface direction at the exit end (26).

23. Apparatus according to any one of claims 18 to 22, wherein the casting surface (20) comprises the peripheral surface of a rotating casting wheel.

24. Apparatus according to claims 22 and 23, wherein the exit end (26) of the vessel (18) is adjacent a position on the casting wheel forming an angle of 0°-45°.

25. Apparatus according to claim 23 or 24, wherein the exit end (26) of the casting vessel (18) is adjacent a position in an upper quadrant of the casting wheel.

26. Apparatus for directly casting molten metal to continuous strip of crystalline material, comprising a casting vessel (18) having an exit (26) and a casting surface (20) movable generally upwardly past the exit (26) characterised in:
the casting vessel (18) being substantially horizontal and having a receiving end (22), an exit end (26) having a generally U-shaped structure adjacent the casting surface (20) and substantially parallel thereto, and an intermediate section (24) communicating between the receiving end (22) and the exit end (26), the intermediate section (24) having a gradually increasing width to the exit end (26) and a gradually decreasing depth to the exit end (26) so as to maintain at least a substantially uniform cross-sectional area or greater from the receiving end (22) to the exit end (26) of the vessel (18),
the exit end (26) having a bottom wall (28) and sidewalls (30) with diverging inside surfaces (31) opening upwardly and defining the U-shaped structure, the width between the inside surfaces (31) of the sidewalls (30) being substantially as wide as the strip (15) to be cast, the width of the bottom wall (28) between the inside surface (31) of the sidewalls (30) being fixed to provide a substantially uniform cross-sectional area over a length at least equal to the depth of the molten metal (19) therein, the length being sufficient to provide a substantially uniform flow of molten metal from the exit end (26),
said casting surface (20) being movable generally upwardly past the exit end (26) of the casting vessel (18) at a distance of between 0.005 to 0.060 inches (0.127 to 1.524 mm) therefrom and said surface (20) having an upward path forming an angle of 0 to 135° between the direction of metal flow at the free surface and the direction of casting surface movement, the casting surface (20) moving at a speed of 20 to 500 feet (6.096 to 152.4 metres) per minute.

## Patentansprüche

1. Verfahren zum direkten Gießen einer Metallschmelze in ein kontinuierliches Band aus kristallinem Metall, welches umfaßt:
Zuführen der Metallschmelze (19) zu einem Gießgefäß (18), Bewegen einer gekühlten Gießfläche (20) im allgemeinen aufwärts hinter einem Ende des Gießgefäßes, Strömen der Metallschmelze von dem Ausgang auf die bewegte Gießfläche, wobei die Oberflächenspannung der freien Oberfläche der Metallschmelze eine Meniskus (35) zwischen dem Ausgang und der Gießfläche aufrechterhält, und Abnehmen des Gießbandes (15) von der bewegten Gießfläche, gekennzeichnet durch
das Gießgefäß (18) mit einem Aufnahmeende (22) und einem Ausgangsende (26), wobei das Ausgangsende (26) nahe der Gießfläche (20) angeordnet ist und parallel zur Gießfläche (20) angeordnete Kanten (33) aufweist;
Zuführen der Metallschmelze von Aufnahmeende (22) zum Ausgangsende (26), um ein Metallschmelzbecken mit einer im wesentlichen gleichförmigen Strömung und einer freien oberen Fläche am Ausgangsende (26) des Gießgefäßes (18) zu schaffen;
Strömen der Metallschmelze vom Ausgangsende (26) auf die bewegte Gießfläche (20) mit einer im wesentlichen gleichförmigen Strömung quer zur Breite des Ausgangsendes (26), wobei die Oberflächenspannung des strömenden Metalls alle Flächen des zu gießenden Bandes formt, die Oberflächenspannung der freien Fläche des Metallschmelzbeckens die Oberseite des Gießbandes ausbildet, der Meniskus (35) den Boden des Gießbandes formt; die Oberflächenspannung der zwei Seiten (30) des Ausgangsendes (26) verlassenden Metallschmelze die Kanten des Gießbandes formt, die im wesentlichen ebenso breit wie das gegossene Band sind; und
Steuern der Tiefe der Metallschmelze im Ausgangsende (26) des Gefäßes (18) und des Abstandes zwischen dem Ausgangsende (26) und der Gießfläche (20), um die Oberflächenspannung der Metallschmelze an der Oberseite, dem Boden und den Seiten aufrechtzuerhalten.

2. Verfahren nach Anspruch 1, wobei das Zuführen der Metallschmelze (19) vom Aufnahmeende (22) zum Ausgangsende (26) ein Aufrechterhalten eines im wesentlichen gleichförmigen Strömungsquerschnitts im Ausgangsende (26) umfaßt.

3. Verfahren nach Anspruch 1 oder 2, wobei das Zuführen der Metallschmelze (19) das Aufrechterhalten eines im wesentlichen gleichförmigen Strömungsquerschnitts vom Aufnahmeende (22) durch das Ausgangsende (26) umfaßt.

4. Verfahren nach Anspruch 1, oder 3, wobei das Zuführen der Metallschmelze (19) in dem Gießgefäß (18) das Vorsehen einer -Metallschmelze in dem Aufnahmeende (22) bei gleichem Niveau wie am Ausgangsende (26) umfaßt.

5. Verfahren nach einem der vorhergehenden Ansprüche, wobei das Zuführen der Metallschmelze (19) ein allmähliches Ansteigen der Strömungsbreite vom Aufnahmeende (22) zum Ausgangsende (26) umfaßt, während ein im wesentlichen gleichformiger Strömungsquerschnitt beibehalten wird.

6. Verfahren nach einem der vorhergehenden Ansprüche, welches ein Leiten der Metallschmelzströmung in dem Gießgefäß (18) umfaßt, um die Entwicklung einer gleichförmigen Strömung am Ausgangsende (26) zu erleichtern.

7. Verfahren nach einem der vorhergehenden Ansprüche, welches ein Bewegen der Gießfläche (20) hinter einer im allgemeinen U-förmigen Struktur des Ausgangsendes (26) des Gefäßes (18) in eine im allgemeinen vom Boden der U-förmigen Konstruktion zur Oberseite des Ausgangsendes (26) weisenden Richtung umfaßt.

8. Verfahren nach einem der vorhergehenden Ansprüche, welches das Bewegen der Gießfläche (20) auf einem Weg von der Horizontalen in die Richtung der Metallströmung bei einem zwischen der freien Oberfläche und der Richtung der Gießfläche am Ausgangsende (26) des Gefäßes (18) ermittelten Winkel von 0° bis 135° umfaßt.

9. Verfahren nach Anspruch 8, wobei der Winkel von der Horizontalen zwischen 0° und 45° beträgt.

10. Verfahren nach einem der vorhergehenden Ansprüche, welches ein Steuern der Dicke des Bandes (15) durch die Geschwindigkeit der Gießfläche (20) und der Tiefe der Metallschmelze (19) am Ausgangsende (26) des Gießgefäßes (18) umfaßt.

11. Verfahren nach einem der vorhergehenden Ansprüche, welches ein Kühlen der Metallschmelze nach dem Kontakt mit der Gießfläche (20) bei einer Geschwindigkeit von weniger als 2000°C/sek. umfaßt, um eine Verfestigung des kristallinen Metalls zu bewirken.

12. Verfahren nach Anspruch 11, wobei das Kühlen bei einer Geschwindigkeit von weniger als 1500°C/sek. erfolgt.

13. Verfahren nach einem der vorhergehenden Ansprüche, wobei die Gießfläche mit einer Geschwindigkeit von 20 bis 500 Fuß/min. (6,096 bis 152,4 m/min.) bewegt wird.

14. Verfahren nach einem der vorhergehenden Ansprüche, welches das Vorsehen der Gießfläche (20) parallel zu Kanten (33) des Ausgangsendes (26) bei einem Abstand zwischen 0,005 bis 0,060 inch (0,127 bis 1,524 mm) vom Ausgangsende (26) umfaßt.

15. Verfahren nach einem der vorhergehenden Ansprüche, welches ein Abnehmen des Bandes (15) von der Gießfläche (20) umfaßt, das eine gleichförmige Bandbreite aufweist, die zwischen 4 und 48 inch (10,16 bis 121,92 cm) liegt.

16. Verfahren nach einem der vorhergehenden Ansprüche, welches des Abnehmen des Bandes (15) von der Gießfläche (20) umfaßt, das eine gleichförmige Dicke aufweist, die zwischen 0,010 und 0,100 inch (0,254 und 2,54 mm) liegt.

17. Verfahren zum direkten Gießen einer Metallschmelze in ein kontinuierliches Band aus kristallinem Metall, welches umfaßt: Zuführen der Metallschmelze (19) zu einer Gießgefäß (18), Bewegen einer gekühlten Gießfläche (20) im allgemeinen aufwärts hinter einem Ausgang des Gießfäßes, Strömen der Metallschmelze von dem Ausgang auf die bewegte Gießfläche, wobei die Oberflachenspannung der freien Oberfläche der Metallschmelze einen Meniskus (35) zwischen dem Ausgang und der Gießfläche aufrechterhält, und Abnehmen des Gießbandes (15) von der bewegten Gießfläche, gekennzeichnet durch,
das Gießgefäß (18), welches im wesentlichen horizontal angeordnet ist und ein Aufnahmeende (22) und ein Ausgangsende (26) aufweist, wobei das Ausgangsende (26) nahe einer Gießfläche (20) angeordnet und im allgemeinen U-förmige mit Kanten (33) ausgebildet ist, die sich parallel zur Gießfläche (20) erstrecken und davon mit einem Abstand zwischen 0,005 und 0,060 inch (0,127 bis 1,524 mm) beabstandet sind;
Bewegen der Gießfläche (20) im allgemeinen aufwärts hinter dem Ausgangsende (26) mit einer Geschwindigkeit von 20 bis 500 Fuß/min. (6,096 bis 152,4 m/min.) auf einem Weg bei einem zwischen der freien Oberfläche in Richtung der Metallströmung und der Richtung der Gießfläche (20) am Ausgangsende (26) des Gießgefäßes (18) ermittelten Winkel von 0° bis 135°;
Zufüuhren der Metallschmelze (19) vom Aufnahmeende (22) zum Ausgangsende (26), während ein im wesentlichen gleichförmiger oder größerer Strömungsquerschnitt erhalten wird, um ein Metallschmelzbecken mit einer im wesentlichen gleichförmigen Strömung und einer freien oberen Fläche im Ausgangsende (26) zu schaffen;
Strömen der Metallschmelze (19) von der U-förmigen Konstruktion des Ausgangsendes (26) auf die bewegte Gießfläche (20) mit einer im wesentlichen gleichförmigen Strömung quer zur Breite des Ausgangsendes (26), wobei die Oberflächenspannung des strömenden Metalls die Oberflächen des gegossenen Bandes (15) formt, die Oberflächenspannung der freien Oberfläche der strömenden Metallschmelze die Oberseite des Gießbandes formt, die Oberflächenspannung der zwei Seiten (30) des Ausgangsendes (26) verlassenden Metallschmelze die Kanten des Gießbandes formt, die im wesentlichen die gleiche Breite wie das zu gießende Band (15) aufweisen, und die Oberflächenspannung der den Boden der U-förmigen Struktur verlassenden Metallschmelze den Meniskus (35) zwischen einer Innenfläche des Bodens (28) des Ausgangsendes (26) und der Gießfläche (20) aufrechterhält, um den Boden des Gießbandes (15) zu formen;
Kühlen der Metallschmelze durch Kontakt mit der Gießfläche (20) mit einer Geschwindigkeit von weniger als 2000°C/sek., um ein Verfestigen des kristallinen Metalls zu bewirken; und
Steuern der Tiefe der Metallschmelze im Ausgangsende (26) des Gefäßes (18) und des Abstands zwischen dem Ausgangsende (26) und der Gießfläche (20), um die Oberflächenspannung der Metallschmelze an der Oberseite, dem Boden und den Seiten aufrechtzuerhalten.

18. Vorrichtung zum direkten Gießen einer Metallschmelze in ein kontinuierliches Band aus kristallinem Metall, welche umfaßt ein Gießgefäß (18) mit einem Ausgang (26) und eine im allgemeinen aufwärts hinter dem Ausgang (26) bewegbare Gießfläche (20), gekennzeichnet durch:
das Gießgefäß (18) mit einem Aufnahmeende (22), einem im allgemeinen U-förmigen Ausgangsende (26) und einem dazwischen angeordneten Zwischenabschnitt (24);
einer Einrichtung (12) zum Zuführen der Metallschmelze (19) zum Aufnahmeende (22) des Gießgefäßes (18);
das Gießgefäß (18) mit seinem nahe der Gießfläche (20) angeordneten Ausgangsende (26) und im wesentlichen parallel zur Gießfläche (20) angeordneten Kanten (33), dem Zwischenabschnitt (24) zum Erleichtern einer im wesentlichen gleichförmigen Strömung der Metallschmelze (19) von Aufnahmeende (22) zum Ausgangsende (26), dem U-förmigen Ausgangsende (26), das eine ebene Bodenwand (28) und divergierende innere Seitenwände (31) aufweist, die sich aufwärts öffnen und eine Breite zwischen den Innenflächen aufweisen, die derjenigen des zu gießenden Bandes (15) entspricht, einem Ausgangsende (26) mit einer bestimmten Breite entlang der Bodenwand (28) zwischen den Innenflächen (31) der Seitenwände (30) und einem gleichmäßigen Querschnitt über eine Länge, die ausreicht, um eine im wesentlichen gleichförmige Strömung der Metallschmelze vom Ausgangsende (26) zu schaffen;
die im allgemeinen aufwärts hinter dem Ausgangsende (26) des Gießgefäßes (18) mit einem Abstand davon zwischen 0,005 und 0,060 inch (0,127 und 1,524 mm) mit einer Geschwindigkeit von 20 bis 500 Fuß/min. (6,096 bis 152,4 m/min.) bewegbare Kühlfläche (20).

19. Vorrichtung nach Anspruch 18, welche ein Gießgefäß (18) umfaßt, wobei das Niveau der Metallschmelze im Aufnahmeende (22) dasselbe ist wie im Ausgangsende (26).

20. Vorrichtung nach Anspruch 18 oder 19, wobei der das Aufnahmeende (22) und das Ausgangsende (26) verbindende Zwischenabschnitt (24) eine allmählich ansteigende Breite am Ausgangsende (26) und eine allmählich sich verringernde Tiefe aufweist, um einen im wesentlichen gleichförmigen Querschnitt längs des Gießgefäßes (18) zu erhalten.

21. Vorrichtung nach Anspruch 18, 19 oder 20, welche Leitwände (36, oder 48, 50) im Gießgefäß (18) umfaßt, um die Entwicklung einer gleichförmigen Strömung zu erleichtern.

22. Vorrichtung nach einem der vorhergehenden Ansprüche 18 bis 21, wobei die Gießfläche (20) eine Bewegungsrichtung aufwärts von der Horizontalen und eine Metallströmrichtung an der freien Oberfläche der Metallschmelze am Ausgangsende (26) aufweist, die unter einem Winkel von 0 bis 135° zur Horizontalen zwischen der freien Oberfläche und der Gießflächenrichtung am Ausgangsende (26) ausgerichtet ist.

23. Vorrichtung nach einem der Ansprüche 18 bis 22, wobei die Gießfläche (20) die Umfangsfläche eines rotierenden Gießrades aufweist.

24. Vorrichtung nach den Ansprüchen 22 und 23, wobei das Ausgangsende (26) des Gefäßes (18) nahe einer einen Winkel von 0° bis 45° bildenden Position auf dem Gießrad angeordnet ist.

25. Vorrichtung nach Anspruch 23 oder 24, wobei das Ausgangsende (26) des Gießgefäßes (18) nahe einer Position in einem oberen Quadranten des Gießrades angeordnet ist.

26. Vorrichtung zum direkten Gießen einer Metallschmelze in ein kontinuierliches Band aus kristallinem Material, welche umfaßt ein Gießgefäß (18) mit einem Ausgang (26) und eine im allgemeinen aufwärts hinter dem Ausgang (26) bewegbare Gießfläche (20), gekennzeichnet durch:
das im wesentlichen horizontal angeordnete Gießgefäß (18) mit einem Aufnahmeende (22), einem Ausgangsende (26) mit einer im wesentlichen U-förmigen, nahe der Gießfläche (20) und im wesentlichen parallel dazu angeordneten Struktur und einem das Aufnahmeende (22) und das Ausgangsende (26) verbindenden Zwischenabschnitt (24), der eine allmählich zum Ausgangsende (26) ansteigende Breite und eine allmählich zum Ausgangsende (26) abnehmende Tiefe aufweist, um wenigstens einen im wesentlichen gleichförmigen oder größeren Querschnitt vom Aufnahmeende (22) zum Ausgangsende (26) des Gefäßes (18) zu erhalten,
das Ausgangsende (26) mit einer Bodenwand (28) und Seitenwänden (30) mit divergierenden Innenflächen (33), die sich nach oben öffnen und die U-förmige Struktur festlegen, wobei die Breite zwischen den Innenflächen (31) der Seitenwände (30) im wesentlichen derjenigen des zu gießenden Bandes (15) entspricht, die Breite der Bodenwand (28) zwischen der Innenfläche (31) der Seitenwände (30) festgelegt ist, um einen im wesentlichen gleichförmigen Querschnitt über eine Länge zu schaffen, die wenigstens der Tiefe der darin befindlichen Metallschmelze (19) entspricht und dazu ausreicht, eine im wesentlichen gleichförmige Metallschmelzströmung vom Ausgangsende (26) zu schaffen,
die Gießfläche (20), welche im allgemeinen aufwärts hinter dem Ausgangsende (26) des Gießgefäßes (18) mit einem Abstand davon zwischen 0,005 und 0,060 inch (0,127 und 1,524 mm) bewegbar ist und einen aufwärts gerichteten Weg aufweist, welcher einen Winkel von 0 bis 135° zwischen der Metallströmrichtung an der freien Oberfläche und der Bewegungsrichtung der Gießfläche ausbildet, wobei die Gießfläche (20) bei einer Geschwindigkeit von 20 bis 500 Fuß/min. (6,096 bis 152,4 m/min.) bewegt wird.

## Revendications

1. Procédé de coulée directe d'un métal fondu sous forme d'une bande continue d'un métal cristallin, comprenant la transmission d'un métal fondu (19) à un réservoir de coulée (18), le déplacement d'une surface de coulée et de refroidissement (20) en direction générale ascendante devant une sortie du réservoir de coulée, l'écoulement du métal fondu de la sortie sur la surface mobile de coulée, les forces de tension superficielle deula surface libre du métal fondu assurant le maintien d'un ménisque (35) entre la sortie et la surface de coulée, et l'enlèvement de la bande coulée (15) de la surface mobile de coulée, caractérisé en ce que:

le réservoir de coulée (18) a une extrémité de réception (22) et une extrémité de sortie (26), l'extrémité de sortie (26) étant adjacente à la surface de coulée (20) et ayant des bords (33) qui sont parallèles à la surface de coulée (20), le procédé comprenant:
la transmission du métal fondu de l'extrémité de réception (22) à l'extrémité de sortie (26) afin qu'un bain de métal fondu forme un courant sensiblement uniforme et une surface supérieure libre vers l'extrémité de sortie (26) du réservoir de coulée (18),
l'écoulement du métal fondu depuis l'extrémité de sortie (26) sur la surface mobile de coulée (20), avec formation d'un courant sensiblement uniforme sur toute la largeur de l'extrémité de sortie (26), la tension superficielle du métal qui s'écoule assurant la mise en forme de toutes les surfaces de la bande à couler, la tension superficielle de la surface libre du bain de métal fondu assurant la mise en forme de la partie supérieure de la bande coulée, le ménisque (35) assurant la mise en forme du fond de la bande coulée, la tension superficielle du métal fondu quittant les deux côtés (30) de l'extrémité de sortie (26) assurant la mise en forme des bords de la bande coulée et ayant une largeur sensiblement égale à celle de la bande coulée, et
le réglage de l'épaisseur du métal fondu à l'extrémité de sortie (26) du réservoir (18) et de la distance comprise entre l'extrémité de sortie (26) et la surface de coulée (20) afin que la tension superficielle du métal fondu soit conservée à la partie supérieure, à la partie inférieure et sur les côtés.

2. Procédé selon la revendication 1, dans lequel la transmission du métal fondu (19) de l'extrémité de réception (22) vers l'extrémité de sortie (26) comprend le maintien d'une section pratiquement uniforme d'écoulement vers l'extrémité de sortie (26).

3. Procédé selon la revendication 1 ou 2, dans lequel la transmission du métal fondu (19) comporte le maintien d'une section pratiquement uniforme d'écoulement depuis l'extrémité de réception (22) et par l'intermédiaire de l'extrémité de sortie (26).

4. Procédé selon la revendication 1, ou 3, dans lequel la transmission du métal fondu (19) au réservoir de coulée (18) comprend la transmission de métal fondu à l'extrémité de réception (22) au même niveau qu'à l'extrémité de sortie (26).

5. Procédé selon l'une quelconque des revendications précédentes, dans lequel la transmission du métal fondu (19) comprend la formation d'une largeur d'écoulement croissant progressivement de l'extrémité de recéption (22) vers l'extrémité de sortie (26), avec maintien d'une section sensiblement uniforme d'écoulement.

6. Procédé selon l'une quelconque des revendications précédentes, comprenant le cloisonnement du courant de métal fondu dans le réservoir de coulée (18) afin que la formation d'un courant uniforme à l'extrémité de sortie (26) soit facilitée.

7. Procédé selon l'une quelconque des revendications précédentes, comprenant le déplacement de la surface de coulée (20) devant une structure de forme générale en U de l'extrémité de sortie (26) du réservoir (18), en direction allant de façon générale de la partie inférieure de la structure en U vers la partie supérieure de l'extrémité de sortie (26).

8. Procédé selon l'une quelconque des revendications précédentes, comprenant le déplacement de la surface de coulée (20) suivant un trajet partant d'un plan horizontal et ayant la direction d'écoulement du métal, faisant un angle compris entre 0 et 135°, mesuré entre la surface libre et la direction de la surface de coulée à l'extrémité de sortie (26) du réservoir (18).

9. Procédé selon la revendication 8, l'angle formé avec le plan horizontal est comprise entre 0 et 45°.

10. Procédé selon l'une quelconque des revendications précédentes, comprenant le réglage de l'épaisseur de la bande (15) en fonction de la vitesse de la surface de coulée (20) et de la profondeur du métal fondu (19) à l'extrémité de sortie (26) du réservoir de coulée (18).

11. Procédé selon l'une quelconque des revendications précédentes, comprenant le refroidissement du métal fondu après son contact avec la surface de coulée (20) à une vitesse inférieure à 2 000°C/s afin qu'un métal cristallin se solidifie.

12. Procédé selon la revendication 11, dans lequel le refroidissement est réalisé à une vitesse inférieure à 1 500°C/s.

13. Procédé selon l'une quelconque des revendications précédentes, dans lequel la surface de coulée est déplacée à une vitesse comprise entre 6,096 et 152,4 m/min (20 et 500 pieds par minute).

14. Procédé selon l'une quelconque des revendications précédentes, comprenant la disposition de la surface de coulée (20) parallèlement aux bords (33) de l'extrémité de sortie (26) et à une distance de 0,127 et 1,524 mm (0,005 à 0,060 pouce) de l'extrémité de sortie (26).

15. Procédé selon l'une quelconque des revendications précédentes, comprenant l'enlèvement de la bande (15) de la surface de coulée (20) avec une largeur uniforme de bande, comprise entre 10,16 et 121,92 cm (4 et 48 pouces).

16. Procédé selon l'une quelconque des revendications précédentes, comprenant l'enlèvement de la bande (15) de la surface de coulée (20) avec une épaisseur uniforme qui est comprise entre 0,254 et 2,54 mm (0,010 et 0,100 pouce).

17. Procédé de coulée directe d'un métal fondu sous forme d'une bande continue d'un métal cristallin, comprenant la transmission de métal fondu (19) à un réservoir de coulée (18), le déplacement d'une surface de coulée et de refroidissement (20) en direction générale ascendante devant une sortie du réservoir de coulée, l'écoulement du métal fondu de la sortie sur la surface mobile de coulée, la tension superficielle de la surface libre du métal fondu assurant l'entretien d'un ménisque (35) entre la sortie et la surface de coulée, et l'enlèvement de la bande coulée (15) de la surface mobile de coulée, caractérisé en ce que:
le réservoir de coulée (18) est pratiquement horizontal et a une extrémité de réception (22) et une extrémité de sortie (26), l'extrémité de sortie (26) étant adjacente à une surface de coulée (20) et ayant une forme générale en U avec des bords (33) qui sont parallèles à la surface de coulée (20) et qui sont séparés de celle-ci par une distance comprise entre 0,127 et 1,524 mm (0,005 et 0,060 pouce), le procédé comprenant:
le déplacement de la surface de coulée (20) en direction générale ascendante devant l'extrémité de sortie (26) à une vitesse comprise entre 6,096 et 152,4 m/min (20 et 500 pieds par minute) suivant un trajet faisant un angle de 0 à 135°, mesuré entre la surface libre, dans la direction d'écoulement du métal, et la direction de la surface de coulée (20) à l'extrémité de sortie (26) du réservoir de coulée (18),
la transmission du métal fondu (19) de l'extrémité de réception (22) à l'extrémité de sortie (26) avec conservation d'une section pratiquement uniforme ou accrue afin qu'un bain de métal fondu ayant un débit sensiblement uniforme et ayant une surface supérieure libre à l'extrémité de sortie (26) soit formé,
l'écoulement du métal fondu (19) de la structure en U de l'extrémité de sortie (26) sur la surface mobile de coulée (20) avec un débit sensiblement uniforme sur la largeur de l'extrémité de sortie (26), la tension superficielle du métal qui s'écoule assurant la mise en forme des surfaces de la bande (15) qui est coulée, la tension superficielle de la surface libre du métal fondu qui s'écoule formant la partie supérieure de la bande coulée, la tension superficielle du métal fondu quittant les deux côtés (30) à l'extrémité de sortie (26) formant les bords de la bande coulée et ayant une largeur pratiquement égale à celle de la bande (15) qui est coulée, la tension superficielle du métal fondu quittant le fond de la structure en U assurant l'entretien du ménisque (35) entre la surface interne du fond (28) de l'extrémité de sortie (26) et la surface de coulée (20) afin que le fond de la bande coulée (15) soit formé,
le refroidissement du métal fondu au contact de la surface de coulée (20) à une vitesse inférieure à 2 000°C/s afin que le métal cristallin se solidifié, et
le réglage de la profondeur du métal fondu à l'extrémité de sortie (26) du réservoir (18) et de la distance comprise entre l'extrémité de sortie (26) et la surface de coulée (20) afin que la tension superficielle du métal fondu soit conservée à la partie supérieure, à la. partie inférieure et sur les côtés.

18. Appareil de coulée directe de métal fondu sous forme d'une bande continue d'un matériau cristallin, comprenant un réservoir de coulée (18) ayant une sortie (26) et une surface de coulée (20) mobile en direction générale ascendante devant la sortie (26), caractérisé en ce que:
le réservoir de coulée (18) a une extrémité de réception (22), une extrémité de sortie (26) de forme générale en U et un tronçon intermédiaire (24), et
un dispositif (12) destiné à transmettre du métal fondu (19) à l'extrémité de réception (22) du réservoir de coulée (18),
le réservoir de coulée (18) ayant une extrémité de sortie (26) qui est adjacente à la surface de coulée (20) et dont les bords (33) sont pratiquement parallèles à la surface de coulée (20), le tronçon intermédiaire (24) facilitant l'écoulement sensiblement uniforme du métal fondu (19) de l'extrémité de réception (22) à l'extrémité de sortie (26), l'extrémité de sortie en U (26) ayant une paroi inférieure plane (28) et des parois latérales internes (31) qui divergent, débouchant vers le haut et ayant une largeur, comprise entre les surfaces internes, qui est sensiblement égale à celle de la bande (15) à couler, l'extrémité de sortie (26) ayant une largeur fixe le long de la paroi inférieure (28) entre les surfaces internes (31) des parois latérales (30) et une section uniforme sur une longueur suffisante pour qu'un courant sensiblement uniforme de métal fondu soit formé à l'extrémité de sortie (26),
la surface de coulée (20) étant mobile en direction générale ascendante devant l'extrémité de sortie (26) du réservoir de coulée (18) à une distance de l'extrémité qui est comprise entre 0,127 et 1,524 mm (0,005 et 0,60 pouce), à une vitesse comprise entre 6,096 et 152,4 m/min (200 et 500 pieds par minute).
19. Appareil selon la revendication 18, comprenant un réservoir de coulée (18) dans lequel les niveaux du métal fondu à l'extrémité de réception (22) et à l'extrémité de sortie (26) sont les mêmes.

20. Appareil selon la revendication 18 ou 19, dans lequel le tronçon intermédiaire (24) communiquant avec l'extrémité de réception (22) et l'extrémité de sortie (26) a une largeur croissant progressivement vers l'extrémité de sortie (26) et une profondeur décroissant linéairement de manière qu'une section pratiquement uniforme soit conservée sur toute la longueur du réservoir de coulée (18).

21. Appareil selon la revendication 18,19 ou 20, comprenant des déflecteurs (36 ou 48, 50) placés dans le réservoir de coulée (18) et destinés à faciliter la création d'un courant uniforme.

22. Appareil selon l'une quelconque des revendications précédentes 18 à 21, dans lequel la surface de coulée (20) a une direction ascendante de déplacement à partir du plan horizontal, et la direction du métal fondu, à la surface libre du métal fondu à l'extrémité de sortie (26), est orientée avec une inclinaison comprise entre 0 et 135° par rapport au plan horizontal, cet angle étant comprise entre la surface libre et la direction de la surface de coulée à l'extrémité de sortie (26).

23. Appareil selon l'une quelconque des revendications 18 à 22, dans lequel la surface de coulée (20) est la surface périphérique d'une roue rotative de coulée.

24. Appareil selon les revendications 22 et 23, dans lequel l'extrémité de sortie (26) du reservoir (18) est adjacente à un emplacement de la roue de coulée qui forme un angle compris entre 0 et 45°.

25. Appareil selon la revendication 23 ou 24, dans lequel l'extrémité de sortie (26) du réservoir de coulée (18) est adjacente à un emplacement compris dans un quadrant supérieur de la roue de coulée.

26. Appareil de coulée directe d'un métal fondu sous forme d'un bande continue d'un matériau cristallin, comprenant un réservoir de coulée (18) ayant une sortie (26) et une surface de coulée (20) mobile en direction générale ascendante devant la sortie (26), caractérisé en ce que:
le réservoir de coulée (18) est sensiblement horizontal et a une extrémité de réception (22), une extrémité de sortie (26) ayant une structure de forme générale en U, adjacente à la surface de coulée (20) et sensiblement parallèle à celle-ci, et un tronçon intermédiaire (24) assurant la communication entre l'extrémité de réception (22) et l'extrémité de sortie (26), le tronçon intermédiaire (24) ayant une largeur croissant progressivement vers l'extrémité de sortie (26) et une profondeur décroissant progressivement vers l'extrémité de sortie (26) afin qu'une section au moins sensiblement uniforme ou croissante soit obtenue de l'extrémité de réception (22) vers l'extrémité de sortie (26) du reservoir (18),
l'extrémité de sortie (26) ayant une paroi inférieure (28) et des parois latérales (30) ayant des surfaces internes (31) qui divergent, débouchant vers le haut et délimitant la structure en U, la largeur mesurée entre les surfaces internes (31) des parois latérales (30) étant pratiquement égale à celle de la bande (15) qui doit être coulée, la largeur de la paroi inférieure (28) comprise entre la surface interne (31) des parois latérales (30) étant fixe afin qu'elle détermine une section sensiblement uniforme sur une longueur au moins égale à la largeur de métal fondu (19) à l'intérieur, la longueur étant suffisante pour qu'un courant sensiblement uniforme de métal soit formé à partir de l'extrémité de sortie (26),
la surface de coulée (20) étant mobile en direction générale ascendante en face de l'extrémité de sortie (26) du réservoir de coulée (18) à une distance comprise entre 0,127 et 1,524 mm (0,005 et 0,060 pouce) de celle-ci, cette surface (20) ayant une trajectoire ascendante formant un angle de 0 à 135° mesuré entre la direction d'écoulement du métal à la surface libre et la direction de déplacement de la surface de coulée, la surface de coulée (20) se déplaçant à une vitesse de 6,096 à 152,4 m/min (20 à 500 pieds par minute).
